



US009256147B2

(12) **United States Patent**  
**Yamaguchi et al.**

(10) **Patent No.:** **US 9,256,147 B2**  
(b5) **Date of Patent:** **\*Feb. 9, 2016**

- (54) **TONER, AND IMAGE FORMING METHOD AND PROCESS CARTRIDGE USING THE TONER**
- (71) Applicant: **RICOH COMPANY, LTD.**, Ohta-Ku, Tokyo (JP)
- (72) Inventors: **Hideyuki Yamaguchi**, Numazu (JP); **Hachiroh Tosaka**, Numazu (JP); **Tomoyuki Satoh**, Numazu (JP)
- (73) Assignee: **RICOH COMPANY, LTD.**, Tokyo (JP)
- (\*) Notice: Subject to any disclaimer, the term of this patent is extended or adjusted under 35 U.S.C. 154(b) by 0 days.
- This patent is subject to a terminal disclaimer.
- (21) Appl. No.: **13/737,230**
- (22) Filed: **Jan. 9, 2013**
- (65) **Prior Publication Data**
- US 2013/0122417 A1 May 16, 2013
- Related U.S. Application Data**
- (62) Division of application No. 11/983,690, filed on Nov. 9, 2007, now Pat. No. 8,372,569.
- (30) **Foreign Application Priority Data**
- Nov. 17, 2006 (JP) ..... 2006-311162  
Sep. 12, 2007 (JP) ..... 2007-236088  
Sep. 20, 2007 (JP) ..... 2007-243514
- (51) **Int. Cl.**
- G03G 9/087* (2006.01)  
*G03G 9/08* (2006.01)  
*G03G 9/097* (2006.01)  
*G03G 13/20* (2006.01)  
*G03G 21/18* (2006.01)
- (52) **U.S. Cl.**
- CPC ..... *G03G 9/0827* (2013.01); *G03G 9/0802* (2013.01); *G03G 9/08753* (2013.01); *G03G 9/09716* (2013.01); *G03G 9/09725* (2013.01); *G03G 13/20* (2013.01); *G03G 21/18* (2013.01)
- (58) **Field of Classification Search**
- CPC ..... G03G 9/0827; G03G 9/0815; G03G 9/09725; G03G 9/08753; G03G 13/08; G03G 13/20
- USPC ..... 430/110.3, 108.7, 109.1, 123.51, 430/123.52, 124.4
- See application file for complete search history.
- (56) **References Cited**
- U.S. PATENT DOCUMENTS**
- |                |         |                                 |
|----------------|---------|---------------------------------|
| 4,401,740 A    | 8/1983  | Kawabata et al.                 |
| 4,670,368 A    | 6/1987  | Tosaka et al.                   |
| 4,762,763 A    | 8/1988  | Nomura et al.                   |
| 5,164,774 A    | 11/1992 | Tomita et al.                   |
| 5,527,657 A    | 6/1996  | Takeda et al.                   |
| 5,840,456 A    | 11/1998 | Tomita et al.                   |
| 5,882,832 A    | 3/1999  | Tosaka et al.                   |
| 6,004,715 A    | 12/1999 | Suzuki et al.                   |
| 6,022,661 A    | 2/2000  | Kurose et al.                   |
| 6,063,537 A    | 5/2000  | Nakamura et al.                 |
| 6,168,894 B1   | 1/2001  | Aoki et al.                     |
| 6,174,641 B1   | 1/2001  | Nakamura et al.                 |
| 6,183,928 B1   | 2/2001  | Sata et al.                     |
| 6,335,138 B1   | 1/2002  | Kurose et al.                   |
| 6,360,068 B1   | 3/2002  | Kinoshita et al.                |
| 6,395,443 B2   | 5/2002  | Kuroda et al.                   |
| 6,416,914 B1   | 7/2002  | Nakamura et al.                 |
| 6,432,589 B1   | 8/2002  | Uchinokura et al.               |
| 6,498,905 B1   | 12/2002 | Tsuruya                         |
| 6,503,676 B2   | 1/2003  | Yamashita et al.                |
| 6,737,210 B2   | 5/2004  | Uchinokura et al.               |
| 6,821,699 B2   | 11/2004 | Kondou et al.                   |
| 6,855,468 B1   | 2/2005  | Yamamoto et al.                 |
| 6,969,574 B1   | 11/2005 | Tosaka et al.                   |
| 7,090,955 B2   | 8/2006  | Tosaka et al.                   |
| 7,250,240 B2   | 7/2007  | Tosaka et al.                   |
| 8,372,569 B2 * | 2/2013  | Yamaguchi et al. .... 430/108.7 |

(Continued)

**FOREIGN PATENT DOCUMENTS**

|    |              |         |
|----|--------------|---------|
| EP | 1 249 735 A2 | 10/2002 |
| EP | 1 439 429 A  | 7/2004  |
| EP | 1 515 193 A  | 3/2005  |

(Continued)

**OTHER PUBLICATIONS**

European Patent Office, extended European search report dated Feb. 6, 2008 in European Patent Application No. 07120312.9-1217, Ricoh Company, Ltd.

Japanese Patent Office, Information Offer Form (Jun. 30, 2010), Japanese Patent Application No. 2007-243514 (Ricoh).

Japanese Patent Office, Office Action dated Aug. 29, 2011 in Japanese Patent Application No. 2007-243514 (Ricoh).

Japanese Patent Office, Office Action dated Jan. 10, 2012 in Japanese Patent Application No. 2007-243514 (Ricoh).

*Primary Examiner* — Janis L Dote

(74) *Attorney, Agent, or Firm* — Cooper & Dunham LLP

**ABSTRACT**

A toner is provided including toner particles A having a circularity of greater than 0.93 and not greater than 1.00 and toner particles B having a circularity of from 0.85 to 0.93, wherein the following relationships are satisfied:  $70 \leq R_A \leq 95$ ,  $5 \leq R_B \leq 30$ ,  $0.014 \leq SD \leq 0.025$ , and  $0.940 \leq ED \leq 0.950$ , wherein  $R_A$  (% by number) represents a ratio of a number of the toner particles A to a total number of toner particles included in the toner,  $R_B$  (% by number) represents a ratio of a number of the toner particles B to the total number of toner particles included in the toner, SD represents a standard deviation of circularity of the toner particles A, and ED represents an average envelope degree of the toner particles B.

---

| (56)                     | <b>References Cited</b> |         |                 |    |                       |
|--------------------------|-------------------------|---------|-----------------|----|-----------------------|
| U.S. PATENT DOCUMENTS    |                         |         |                 |    |                       |
| 2003/0036008             | A1                      | 2/2003  | Yamazaki et al. | JP | 2000-003068 A 1/2000  |
| 2004/0067189             | A1                      | 4/2004  | Sugiura et al.  | JP | 2001-100456 A 4/2001  |
| 2004/0234882             | A1                      | 11/2004 | Matsui et al.   | JP | 2001-100459 A 4/2001  |
| 2005/0079429             | A1                      | 4/2005  | Hayami et al.   | JP | 2001-134015 A 5/2001  |
| 2005/0095516             | A1                      | 5/2005  | Ohmura et al.   | JP | 2001-222132 A 8/2001  |
| 2005/0208398             | A1                      | 9/2005  | Ohmura et al.   | JP | 2002-023409 A 1/2002  |
| FOREIGN PATENT DOCUMENTS |                         |         |                 |    |                       |
| JP                       | 6-067461                | A       | 3/1994          | JP | 2002-107992 A 4/2002  |
| JP                       | 06-148926               |         | 5/1994          | JP | 2002-372802 A 12/2002 |
| JP                       | 08-062893               | A       | 3/1996          | JP | 2004-004507 A 1/2004  |
| JP                       | 09-043909               | A       | 2/1997          | JP | 2004-102236 A 4/2004  |
| JP                       | 09-134027               | A       | 5/1997          | JP | 2004-212789 A 7/2004  |
| JP                       | 10-319622               | A       | 12/1998         | JP | 2005-010723 A 1/2005  |
| JP                       | 2996629                 |         | 10/1999         | JP | 2005-107517 A 4/2005  |
| JP                       | 3009994                 |         | 12/1999         | JP | 2005-157314 A 6/2005  |
| JP                       | 2000-003063             | A       | 1/2000          | JP | 2005-215253 A 8/2005  |
| JP                       |                         |         |                 | JP | 2005-215255 A 8/2005  |
| JP                       |                         |         |                 | JP | 2006-208758 A 8/2006  |
| JP                       |                         |         |                 | JP | 2006-259311 A 9/2006  |
| JP                       |                         |         |                 | JP | 2006-293335 A 10/2006 |
| JP                       |                         |         |                 | JP | 2007-079223 A 3/2007  |
| JP                       |                         |         |                 | JP | 2007-193048 A 8/2007  |

\* cited by examiner

FIG. 1



FIG. 2



FIG. 3



FIG. 4



FIG. 5



FIG. 6



## 1

**TONER, AND IMAGE FORMING METHOD  
AND PROCESS CARTRIDGE USING THE  
TONER**

**CROSS REFERENCE TO RELATED  
APPLICATION**

This application is a division of copending U.S. patent application Ser. No. 11/983,690 filed Nov. 9, 2007.

**BACKGROUND OF THE INVENTION**

**1. Field of the Invention**

The present invention relates to a toner for use in electro-photography. Particularly, the present invention also relates to an image forming method and a process cartridge using the toner.

**2. Discussion of the Related Art**

An electric or a magnetic latent image is generally developed with a toner to become visible. The toner typically comprises colored particles in which a colorant, a charge controlling agent, and other additives are contained in a resin. Toner manufacturing methods are broadly classified into pulverization methods and polymerization methods. The pulverization method includes steps of melt-mixing toner components, such as a colorant, a charge controlling agent, and an offset inhibitor, with a thermoplastic resin so that the toner components are uniformly dispersed in the resin; pulverizing the melt-mixed mixture; and classifying the pulverized mixture.

The pulverization method is capable of providing a toner having desired toner properties to some extent. Cross sections made by the pulverization typically include cracks. When a stress is externally applied to the cracks, ultrafine particles tend to peel off therefrom. In a two-component development process, ultrafine particles tend to be produced from the cross sections (i.e., the surface of the toner particle) and adhere to the surface of a magnetic carrier, due to the application of agitation stress thereto. Thereby, the charging ability of the carrier deteriorates and the toner cannot be charged to the desired level.

In attempting to solve the above problems of the pulverization method, unexamined published Japanese Patent Application No. (hereinafter referred to as JP-A) 09-43909 discloses a suspension polymerization method as a toner manufacturing method. The suspension polymerization method is capable of providing a toner not only including few cracks, but also having a spherical shape and a narrow particle diameter distribution. The use of the spherical toner is capable of improving latent image reproducibility, resulting in producing high quality images. However, such a spherical toner is hardly charged, because the spherical toner tends to slip when triboelectrically-charged by a carrier in a two-component development process. In particular, in a development process in which fresh toner particles are successively supplied, such as a continuous printing of a high-image-proportion image, the fresh toner particles cannot be rapidly charged. Therefore, background fouling in that the background portion of an image is soiled with toner particles tends to be caused.

There is another disadvantage that spherical toner particles are difficult to remove with a cleaning blade when remaining on a photoreceptor. When an image having a low image area proportion is developed or transferred, few toner particles tend to remain on the photoreceptor, which are easily removed. In contrast, when an image having a high image area proportion (such as a photograph) is developed or trans-

## 2

ferred or paper is not efficiently supplied, toner particles which are not transferred and remain on the photoreceptor tend to cause the background fouling. Such remaining toner particles also tend to contaminate a charging roller, configured to contact-charge the photoreceptor, and deteriorate the charging ability thereof.

In attempting to solve the above problems, JP-As 08-62893 and 2007-79223 have disclosed toners in which a polymerization toner and a pulverization toner are mixed. The pulverization toner is mixed as an auxiliary component so that the resultant toner is easily removed with a blade. However, the pulverization toner, which includes cracks, cannot be prevented from producing ultrafine particles and tends to adhere to the carrier. As a result, charging ability of the carrier deteriorates. On the other hand, the polymerization toner, which is a main component of the resultant toner, tends to slip on the surface of the carrier when supplied to a development device. Therefore, the polymerization toner cannot be sufficiently frictionized and cannot be rapidly charged, resulting in causing background fouling. These problems cannot be solved even if the mixing ratio of the polymerization and pulverization toners is varied.

**SUMMARY OF THE INVENTION**

Accordingly, an object of the present invention is to provide a toner capable of producing high quality images for a long period of time.

Another object of the present invention is to provide an image forming method and a process cartridge capable of producing high resolution images.

These and other objects of the present invention, either individually or in combinations thereof, as hereinafter will become more readily apparent can be attained by a toner, comprising:

toner particles A having a circularity of greater than 0.93 and not greater than 1.00; and

toner particles B having a circularity of from 0.85 to 0.93, wherein the following relationships are satisfied:

$$70 \leq R_A \leq 95$$

$$5 \leq R_B \leq 30$$

$$0.014 \leq SD \leq 0.025$$

$$0.940 \leq ED \leq 0.950$$

wherein  $R_A$  (% by number) represents a ratio of a number of the toner particles A to a total number of toner particles included in the toner,  $R_B$  (% by number) represents a ratio of a number of the toner particles B to the total number of toner particles included in the toner, SD represents a standard deviation of circularity of the toner particles A, and ED represents an average envelope degree of the toner particles B; and an image forming method and a process cartridge using the toner.

**BRIEF DESCRIPTION OF THE DRAWINGS**

These and other objects, features and advantages of the present invention will become apparent upon consideration of the following description of the preferred embodiments of the present invention taken in conjunction with the accompanying drawings.

FIG. 1 is an example flow curve obtained by a flowtester to explain how to determine the  $1/2$  method melting temperature;

FIG. 2 is a schematic view for explaining how to determine the envelope degree (based on area) of a typical particle of the toner of the present invention;

FIG. 3 is a schematic view illustrating an embodiment of an image forming apparatus using the image forming method of the present invention;

FIG. 4 is a magnified schematic view illustrating an embodiment of the image forming station of the image forming apparatus illustrated in FIG. 3;

FIG. 5 is a schematic view illustrating an embodiment of the process cartridge of the present invention; and

FIG. 6 is a SEM image ( $\times 1,000$ ) of the toner of the present invention.

### DESCRIPTION OF THE PREFERRED EMBODIMENTS

To achieve such objects, the present invention contemplates the provision of a toner including toner particles A having a circularity of greater than 0.93 and not greater than 1.00 and toner particles B having a circularity of from 0.85 to 0.93, wherein the following relationships are satisfied:

$$70 \leq R_A \leq 95$$

$$5 \leq R_B \leq 30$$

$$0.014 \leq SD \leq 0.025$$

$$0.940 \leq ED \leq 0.950$$

wherein  $R_A$  (% by number) represents the ratio of the number of the toner particles A to the total number of toner particles included in the toner,  $R_B$  (% by number) represents the ratio of the number of the toner particles B to the total number of toner particles included in the toner, SD represents the standard deviation of circularity of the toner particles A, and ED represents the average envelope degree (based on area) of the toner particles B.

When  $R_A$  is too small, reproducibility of a latent image significantly deteriorates. When  $R_A$  is too large, supplied fresh toner particles are insufficiently triboelectrically-charged immediately after being supplied to a development device. When a toner includes toner particles A having a circularity of greater than 0.93 and not greater than 1.00 as main components, and toner particles B having a circularity of from 0.85 to 0.93 as auxiliary components in an amount of from 5 to 30% by number, the problem of insufficient triboelectric-charging of supplied fresh toner particles can be solved. This is because the toner particle A, having a substantially spherical shape, can be prevented from slipping on the surface of a carrier when the toner particle B, having an irregular shape, is present together. As a result, the toner can be sufficiently triboelectrically-charged even immediately after fresh toner particles are supplied to a development device. The toner particle A having a substantially spherical shape easily slips on the surface of a carrier, whereas the toner particle B having an irregular shape hardly slips thereon. Therefore, the toner particle B may have a function of preventing the toner particle A from slipping on the surface of a carrier. When  $R_B$  is too small, the problem of insufficient triboelectric-charging of supplied fresh toner particles cannot be solved. When  $R_B$  is too large, reproducibility of a latent image significantly deteriorates.

In the present invention, the toner particles B have an average envelope degree (based on area) of from 0.940 to 0.950. In other words, the toner particles B have a relatively large envelope degree (based on area) while having a rela-

tively small circularity. Because of having a small circularity, the toner particles B hardly slip on the surface of a carrier and easily adhere thereto. In order to prevent a toner particle from adhering and fixing to the surface of a carrier, the toner particle may have a relatively large envelope degree (based on area), i.e., the toner particle may have a few concavities and convexities on the surface thereof. This is because such toner particle may not be so damaged that ultrafine particles are produced, which tend to fix to the surface of a carrier, even when an impact is externally applied thereto. For the above reasons, the toner of the present invention is capable of being charged to a desired level for a long period of time. When the average envelope degree (based on area) of the toner particles B is too large, the function of the toner particles B of accelerating the triboelectric-charging between a carrier and the toner particles A deteriorates.

In the present invention, the toner particles A have a standard deviation of circularity of from 0.014 to 0.025. In other words, each of the toner particles A has a various shape (e.g., 20 a spherical shape, a bell-like cone shape, a flat shape). Toner particles having a large average circularity and a small standard deviation of circularity tend to cause a problem in that an edge portion of an image is smudged when the image is transferred. This is because such toner particles easily form a 25 close-packed structure and aggregate when a transfer pressure is applied thereto, so that the transfer defects are microscopically occurred. If the toner particles include substantially spherical particles with various shapes, the applied transfer pressure is dispersed among the toner particles, 30 resulting in preventing the occurrence of transfer defect. When the standard deviation of circularity is too large, reproducibility of a latent image (in particular, a thin line image) significantly deteriorates.

Since the toner of the present invention includes toner 35 particles having various shapes, such as a spherical shape, a bell-like cone shape, and a flat shape, the contact area between each of the toner particles is increased. Therefore, high-temperature preservability of the toner tends to deteriorate especially when the toner particles include a resin 40 capable of sharply melting, for the sake of using in a non-contact fixing system. However, this problem can be solved by mixing silica particles having a number average primary particle diameter of from 50 to 200 nm (these silica particles may be hereinafter referred to as large-sized silica particles) 45 with the toner particles, because such large-sized silica particles function as a spacer between toner particles.

In the present invention, the large-sized silica particles 50 preferably have a number average primary particle diameter of from 80 to 200 nm, and more preferably from 100 to 180 nm. When the number average primary particle diameter is too small, the large-sized silica particles may not satisfactorily function as a spacer between the toner particles, resulting 55 in deterioration of high-temperature preservability of the toner. When the number average primary particle diameter is too large, the large-sized silica particles tend to release from the surfaces of the toner particles and cause a filming problem in that silica particles form a film thereof on a carrier, image forming members etc., while functioning as a spacer between the toner particles.

In the present invention, 0.05 to 1.0 parts by weight, and 60 more preferably from 0.1 to 0.5 parts by weight, of the large-sized silica particles are mixed with 100 parts by weight of the toner particles. When the amount of the large-sized silica particles is too small, the large-sized silica particles may not satisfactorily function as a spacer between the toner particles. When the amount of the large-sized silica particles is too 65 large, the large-sized silica particles tend to release from the

surfaces of the toner particles and cause the filming problem and deterioration of the developer. Moreover, such large-sized silica particles tend to prevent toner particles from melting and bonding with each other, resulting in deterioration of glossiness of the resultant image and fixability of the toner.

As mentioned above, silica particles having a number average primary particle diameter ( $R$ ) of from 80 to 200 nm may satisfactorily function as a spacer capable of preventing toner particles from aggregating with each other. In addition, such silica particles may prevent other external additives from burying in the surfaces of toner particles when the toner is preserved in a high-temperature atmosphere or is strongly agitated.

Further, the following relationship is preferably satisfied:

$$R/4 \leq \sigma \leq R$$

wherein  $R$  represents the number average primary particle diameter of silica particles and  $\sigma$  represents the standard deviation of particle diameter distribution of the silica particles.

When the above relationship is satisfied, the silica particles include particles having large, medium, and small particle diameters at an appropriate ratio. The silica particles having a small particle diameter may impart fluidity to the toner, whereas the silica particles having a medium or large particle diameter function as a spacer. Silica particles satisfying the above relationship have much more effective functions as an external additive compared to a mixture of particles having large, medium, and small particle diameters. Silica particles further having a shape factor SF-1 of not greater than 130 and a shape factor SF-2 of not greater than 125, i.e., silica particles having a substantially spherical shape, can improve fluidity of the toner and compatibility between the toner particles and the silica particles so that the silica particles hardly release from the toner particles.

The particle diameters of silica particles (particles of inorganic materials) can be measured using particle diameter distribution measurement instruments such as DLS-700 (manufactured by Otsuka Electronics Co., Ltd.) and COULTER N4 (manufactured by Beckman Coulter, Inc.). Since it is difficult to dissociate secondary aggregates of hydrophobized silica particles, particle diameters of such particles are preferably measured from photographs obtained using a scanning electron microscope (SEM) or a transmission electron microscope (TEM).

When using a SEM, a sample may be evaporated with a metal such as platinum. In order not to transform the sample shape by the evaporation, the evaporated metal layer preferably has a small thickness of about 1 nm or less. Alternatively, a sample may not be evaporated when observed using a high-resolution SEM (e.g., S-5200 manufactured by Hitachi, Ltd.) at a low acceleration voltage of several eV to 10 key.

When using a SEM or TEM, at least 100 particles of a sample are observed and photographed. The photograph is analyzed using an image processing device (e.g., LUZEX manufactured by Nireco Corporation) or an image processing software program to statistically determine the particle diameter distribution and the shape factors SF-1 and SF-2. It is preferable to use LUZEX AP (manufactured by Nireco Corporation) to determine the SF-1 and SF-2 in the present invention. However, the kinds of the image processing device and/or software program, and the SEM and/or TEM are not limited to any particular device.

The shape factors SF-1 and SF-2 are defined by the following equations:

$$SF-1 = (L^2/A) \times (\pi/4) \times 100$$

5

$$SF-2 = (P^2/A) \times (1/4\pi) \times 100$$

wherein  $L$  represents the diameter of the circle circumscribing an image of a particle,  $A$  represents the area of the image of the particle, and  $P$  represents the peripheral length of the image of the particle.

A heat roll fixing method, which is one example of contact heating fixing methods, has been widely used in copiers and printers using electrophotography. However, the heat roll fixing method is unsuitable for producing high definition images formed by dots, because a toner forming the dots is squashed when heat and pressure are applied thereto. Therefore, non-contact heating fixing methods have been mainly used in the field of high-quality and high-speed duplex printing or copying. The non-contact heating fixing methods have a disadvantage that a toner is not strongly fixed because a fixing pressure is not applied thereto. This weak fixation notably occurs when the fixing temperature is decreased so as to produce a matte image having a low glossiness.

The toner of the present invention can be strongly and uniformly fixed even when only a small amount of energy is applied thereto, especially in a method such as the non-contact heating fixing method. This is because the toner of the present invention includes particles having various shapes. In this case, the contact area between each of the toner particles is increased.

Both the toner particles A and B preferably include a polyol resin as a binder resin. When both the toner particles A and B include the same component, the difference in chargeability can be reduced even if they have different shapes. A typical polyol resin has thermal properties suitable for use in non-contact heating fixing methods. In addition, a typical polyol resin has high stiffness compared to other resins. Therefore, a toner using a polyol resin tends not to produce ultrafine particles even if the toner is continuously agitated, and an external additive is hardly buried in the surface of the toner. Such a toner has stable chargeability.

From the viewpoint of imparting environmental stability in charging, fixing stability, color reproducibility, glossiness stability, and resistance to paper curling after fixation to the resultant toner, a polyol resin obtained by capping both ends of an epoxy resin and having a polyoxyalkylene unit in the main chain is preferably used. For example, such a resin is obtainable by reacting an epoxy resin having glycidyl groups on both ends and an alkylene oxide adduct of divalent phenol having glycidyl groups on both ends with a dihalide, an isocyanate, a diamine, a diol, a polyphenol, or a dicarboxylic acid. Among these, a divalent phenol is preferably used in terms of reaction stability. A polyphenol and a polycarboxylic acid are also preferably used in combination with the divalent phenol as long as the reactants do not gelate. Specific examples of the alkylene oxide adduct of divalent phenol having glycidyl groups on both ends include, but are not limited to, reaction products of reactions between ethylene oxide, propylene oxide, butylene oxide, and/or a mixture thereof, and a bisphenol (e.g., bisphenol A, bisphenol F). These reaction products may be further reacted with epichlorohydrin and/or  $\beta$ -methyl epichlorohydrin to have a glycidyl group. In particular, a glycidyl ether of an alkylene oxide adduct of bisphenol A, represented by the following formula, is preferably used:



wherein R represents  $-\text{CH}_2-\text{CH}_2-$ ,



or  $-\text{CH}_2-\text{CH}_2-\text{CH}_2-$ ; and each of n and m independently represents an integer not less than 1, and the sum of n and m is from 2 to 6.

The polyol resin for use in the present invention preferably has a number average molecular weight (Mn) of from 1,000 to 5,000, and more preferably from 1,500 to 3,500, to produce an image having good fixability and glossiness by a non-contact heating method. When the Mn is too small, glossiness of the resultant image may excessively increase and preservability of the resultant toner may deteriorate. When the Mn is too large, glossiness of the resultant image may be too small and the fixability thereof may decrease.

The ratio (Mw/Mn) of the weight average molecular weight (Mw) to the number average molecular weight (Mn) of the polyol resin for use in the present invention is preferably 2.0 to 7.0, and more preferably from 3.0 to 6.0, so as to be used for a non-contact heating fixing method. When the ratio (Mw/Mn) is too large, the toner cannot be well melted when fixed by the non-contact heating fixing method.

The polyol resin for use in the present invention preferably has a glass transition temperature of from 50 to 70°C, and more preferably from 55 to 65°C. When the glass transition temperature is too small, preservability of the resultant toner may deteriorate. When the glass transition temperature is too large, the resultant image may not have a desired glossiness and fixability.

#### (Charge Controlling Agent)

The toner of the present invention may include a charge controlling agent.

Specific examples of the charge controlling agent include any known charge controlling agents such as Nigrosine dyes, triphenylmethane dyes, metal complex dyes including chromium, chelate compounds of molybdcic acid, Rhodamine dyes, alkoxyamines, quaternary ammonium salts (including fluorine-modified quaternary ammonium salts), alkylamides, phosphor and compounds including phosphor, tungsten and compounds including tungsten, fluorine-containing activators, metal salts of salicylic acid and salicylic acid derivatives, and organic boron compounds, but are not limited thereto.

Specific examples of commercially available charge controlling agents include, but are not limited to, BONTRON® N-03 (Nigrosine dyes), BONTRON® P-51 (quaternary ammonium salt), BONTRON® 5-34 (metal-containing azo dye), BONTRON® E-82 (metal complex of oxynaphthoic acid), BONTRON® E-84 (metal complex of salicylic acid), and BONTRON® E-89 (phenolic condensation product), which are manufactured by Orient Chemical Industries Co., Ltd.; TP-302 and TP-415 (molybdenum complex of quaternary ammonium salt), which are manufactured by Hodogaya Chemical Co., Ltd.; COPY CHARGE® PSY VP2038 (quaternary ammonium salt), COPY BLUE® PR (triphenyl methane derivative), COPY CHARGE® NEG VP2036, and

10 COPY CHARGE® NX VP434 (quaternary ammonium salt), which are manufactured by Hoechst AG; LRA-901 and LR-147 (boron complex), which are manufactured by Japan Carl it Co., Ltd.; and compounds such as copper phthalocyanine, perylene, quinacridone, azo pigments, and polymers having a functional group such as a sulfonate group, a carboxyl group, and a quaternary ammonium group.

15 The toner of the present invention preferably includes the charge controlling agent in an amount of from 0.5 to 5.0 parts by weight, more preferably from 0.7 to 3.0 parts by weight, and much more preferably from 0.9 to 2.0 parts by weight, based on 100 parts by weight of the colored particles. When the amount is too small, the resultant toner has too small a charge to be practically used. When the amount is too large, fluidity of the resultant toner and developer deteriorate, resulting in deterioration of the resultant image density.

#### (External Additive)

20 The toner of the present invention may include particles of an inorganic material other than the large-sized silica particles having a number average primary particle diameter of from 80 to 200 nm mentioned above.

25 Specific examples of the inorganic material include, but are not limited to, silica, titanium oxide, alumina, barium titanate, magnesium titanate, calcium titanate, strontium titanate, iron oxide, copper oxide, zinc oxide, tin oxide, quartz sand, clay, mica, sand-lime, diatomaceous earth, chromium oxide, cerium oxide, red iron oxide, antimony trioxide, magnesium oxide, zirconium oxide, barium sulfate, barium carbonate, calcium carbonate, silicon carbide, and silicon nitride.

30 The inorganic material particles preferably have an average primary particle diameter of not greater than 30 nm, in terms of imparting fluidity to the resultant toner. In this case, the resultant toner has good fluidity and uniform chargeability, resulting in preventing the occurrence of toner scattering and background fouling.

35 Specific examples of useable commercially available hydrophobized silica particles having an average primary particle diameter of not greater than 30 nm include, but are not limited to, HDK H 2000, HDK H 2050EP, and HVK 21 (from Clariant Japan K. K.); R972, R974, RX200, RY200, R202, R805, and R812 (from Nippon Aerosil Co., Ltd.); and TS530 and TS720 (from Cabot Corporation).

40 Specific examples of useable commercially available titanium oxide particles include, but are not limited to, P-25 (from Nippon Aerosil Co., Ltd.); STT-30 and STT-65C-S (from Titan Kogyo K. K.); TAF-140 (from Fuji Titanium Industry Co., Ltd.); and MT-150W, MT-500B, and MT-600B (from Tayca Corporation).

45 Specific examples of useable commercially available hydrophobized titanium oxide particles include, but are not limited to, T-805 (from Nippon Aerosil Co., Ltd.); STT-30A and STT-65S-S (from Titan Kogyo K. K.); TAF-500T and TAF-1500T (from Fuji Titanium Industry Co., Ltd.); MT-100S and MT-100T (from Tayca Corporation); and IT-S (from Ishihara Sangyo Kaisha, Ltd.).

50 As mentioned above, these silica and/or titanium oxide particles may be used in combination with the above-mentioned large-sized silica particles having an average primary particle diameter of from 80 to 200 nm.

In the present invention, when the toner includes particles of a plurality of inorganic materials, these inorganic materials preferably have different average primary particle diameters. Since the inorganic material particles are externally mixed with toner particles, the inorganic material particles tend to be gradually buried in the toner particles by application of a load in the development process. When a toner includes particles of two kinds of inorganic materials, particles of an inorganic material having a larger average particle diameter function as a spacer between the surfaces of the toner particles and the surfaces of an image bearing member (i.e., a photoreceptor) and/or a carrier, so that particles of another inorganic material having a smaller average particle diameter are not buried in the surfaces of the toner particles. Therefore, the initial covering condition of the toner particles with the inorganic material particles is maintained for a long period of time, resulting in preventing the occurrence of the filming problem. This effect is easily obtainable when a silica and/or titanium oxide particles are used in combination with the above-mentioned large-sized silica particles having an average primary particle diameter of from 80 to 200 nm.

It is preferable that at least one of the inorganic materials used in the toner is hydrophobized with an organic silane compound. In this case, the resultant toner has good environmental stability and the resultant image has a high image quality without image defect. Of course, all of the inorganic material used in the toner may be hydrophobized.

Specific examples of the hydrophobizing agent include, but are not limited to, organic silane compounds (e.g., dimethyldichlorosilane, trimethylchlorosilane, methyltrichlorosilane, allyldimethyldichlorosilane, allylphenyldichlorosilane, benzylidemethylchlorosilane, bromomethylidemethylchlorosilane,  $\alpha$ -chloroethyltrichlorosilane, p-chloroethyltrichlorosilane, chloromethylidemethylchlorosilane, chloromethyltrichlorosilane, p-chlorophenyltrichlorosilane, 3-chloropropyltrichlorosilane, 3-chloropropyltrimethoxysilane, vinyltriethoxysilane, vinyltrimethoxysilane, vinyl tris( $\beta$ -methoxyethoxy)silane,  $\gamma$ -methacryloxypropyltrimethoxysilane, vinyltriacetoxysilane, divinylidichlorosilane, dimethylvinylchlorosilane, octyltrichlorosilane, decyltrichlorosilane, nonyltrichlorosilane, (4-t-propylphenyl)trichlorosilane, (4-t-butylphenyl)trichlorosilane, diphenyldichlorosilane, dihexyldichlorosilane, dioctyldichlorosilane, dinonyldichlorosilane, didecyldichlorosilane, didodecyldichlorosilane, dihexadecyldichlorosilane, (4-t-butylphenyl)octyldichlorosilane, didecenyldichlorosilane, dinoneyldichlorosilane, di-2-ethylhexyldichlorosilane, di-3,3-dimethylpentylidichlorosilane, trihexylchlorosilane, trioctylchlorosilane, tridecylchlorosilane, dioctylmethylchlorosilane, octyldimethylchlorosilane, (4-t-propylphenyl)diethylchlorosilane, isobutyltrimethoxysilane, methyltrimethoxysilane, octyltrimethoxysilane, trimethoxy(3,3,3-trifluoropropyl)silane, hexamethyldisilazane, hexaethyldisilazane, diethyltetraethylsilazane, hexaphenyldisilazane, hexatolyldisilazane), silicone oils (e.g., dimethyl silicone oil, methylphenyl silicone oil, chlorophenyl silicone oil, methylhydrogen silicone oil, alkyl-modified silicone oil, fluorine-modified silicone oil, polyether-modified silicone oil, alcohol-modified silicone oil, amino-modified silicone oil, epoxy-modified silicone oil, epoxy-polyether-modified silicone oil, phenol-modified silicone oil, carboxyl-modified silicone oil, mercapto-modified silicone oil, acryl-modified silicone oil, methacryl-modified silicone oil,  $\alpha$ -methylstyrene-modified silicone oil), silylation agents, silane coupling agents having a fluorinated alkyl group,

organic titanate coupling agents, and aluminum coupling agents. Among these, the organic silane compounds are preferably used.

The above-mentioned inorganic material particles may be treated with the above hydrophobizing agent to prepare hydrophobized particles of the inorganic materials.

The average primary particle diameter of the inorganic material particles can be measured by the aforementioned method.

10 (Colorant)

Specific examples of the colorants for use in the toner of the present invention include any known dyes and pigments such as carbon black, lampblack, Nigrosine dyes, black iron oxide, NAPHTHOL YELLOW S, HANSA YELLOW (10G, 5G and 15 G), Cadmium Yellow, yellow iron oxide, loess, chrome yellow, Titan Yellow, polyazo yellow, Oil Yellow, HANSA YELLOW (GR, A, RN and R), Pigment Yellow L, BENZIDINE YELLOW (G and GR), PERMANENT YELLOW (NCG), VULCAN FAST YELLOW (5G and R), Tartrazine Lake, Quinoline Yellow Lake, ANTHRAZANE YELLOW BGL, isoindolinone yellow, red iron oxide, red lead, orange lead, cadmium red, cadmium mercury red, antimony orange, Permanent Red 4R, Para Red, Fire Red, p-chloro-o-nitroaniline red, Lithol Fast Scarlet G, Brilliant Fast Scarlet, Brilliant Carmine BS, PERMANENT RED (F2R, F4R, FRL, FRL and F4RH), Fast Scarlet VD, VULCAN FAST RUBINE B, Brilliant Scarlet G, LITHOL RUBINE GX, Permanent Red FSR, Brilliant Carmine 6B, Pigment Scarlet 3B, Bordeaux 5B, Toluidine Maroon, PERMANENT BORDEAUX F2K, HELIO BORDEAUX BL, Bordeaux 10B, BON MAROON LIGHT, BON MAROON MEDIUM, Eosin Lake, Rhodamine Lake B, Rhodamine Lake Y, Alizarine Lake, Thioindigo Red B, Thioindigo Maroon, Oil Red, Quinacridone Red, Pyrazolone Red, polyazo red, Chrome Vermilion, Benzidine Orange, perynone orange, Oil Orange, cobalt blue, cerulean blue, Alkali Blue Lake, Peacock Blue Lake, Victoria Blue Lake, metal-free Phthalocyanine Blue, Phthalocyanine Blue, Fast Sky Blue, INDANTHRENE BLUE (RS and BC), Indigo, ultramarine, Prussian blue, Anthraquinone Blue, Fast Violet B, Methyl Violet Lake, cobalt violet, manganese violet, dioxane violet, Anthraquinone Violet, Chrome Green, zinc green, chromium oxide, viridian, emerald green, Pigment Green B, Naphthol Green B, Green Gold, Acid Green Lake, Malachite Green Lake, Phthalocyanine Green, Anthraquinone Green, titanium oxide, zinc oxide, lithopone, etc. These materials can be used alone or in combination. (Other Additives)

The toner of the present invention may include other additives such as a wax.

50 Any known waxes can be used for the toner of the present invention. Specific examples of the wax include, but are not limited to, polyolefin waxes (e.g., polyethylene waxes, polypropylene waxes), hydrocarbons having a long chain (e.g., paraffin waxes, SASOL waxes), and waxes having a carbonyl group. Among these, waxes having a carbonyl group are preferably used.

55 Specific examples of the waxes having a carbonyl group include, but are not limited to, polyalkanoic acid esters (e.g., carnauba waxes, montan waxes, trimethylolpropane tribenenate, pentaerythritol tetrabehenate, pentaerythritol diacetate dibehenate, glycerin tribehenate, 1,18-octadecanediol distearate); polyalkanol esters (e.g., tristearyl trimellitate, distearyl maleate); polyalkanoic acid amides (e.g., ethylenediamine dibenyl amide); polyalkylamides (e.g., trimellitic acid tristearylamide); and dialkyl ketones (e.g., distearyl ketone). Among these waxes having a carbonyl group, polyalkanoic acid esters are preferably used.

## 11

The wax typically has a melting point of from 40 to 160° C., preferably from 50 to 120° C., and more preferably from 60 to 90° C. When the melting point is too low, thermostable preservability of the resultant toner deteriorates. When the melting point is too high, the wax cannot assist toner particles to melt and fuse with each other when fixed at low temperatures.

The wax preferably has a melt viscosity of from 5 to 1,000 cps, and more preferably from 10 to 100 cps, when measured at a temperature 20° C. higher than the melting point of the wax. When the melt viscosity is too large, the wax cannot assist toner particles to melt and fuse with each other when fixed at low temperatures.

The toner of the present invention preferably has a 1/2 method melting temperature (to be explained in detail later), measured by a flowtester, of from 100 to 115° C., for use in non-contact fixing methods. It is important that the toner has a 1/2 method melting temperature of not greater than 115° C. When the 1/2 method melting temperature is too high, the fixation may be performed at an extremely high temperature, resulting in raising a possibility of causing an ignition of a transfer material. When the 1/2 method melting temperature is too low, the toner tends to cause a filming problem in which a toner forms films thereof on an image bearing member, a carrier, a development sleeve, etc. In order to prevent the occurrence of the filming problem, the toner preferably has a 1/2 method melting temperature of from 100 to 115° C., and more preferably from 105 to 110° C.

When a plurality of toners are used in an image, it is important that each of the toners has a difference in 1/2 method melting temperature of not greater than 10° C. from the other toners. When an image includes two or more toner layers having different colors, the adhesion property between the toner layers may be considered in addition to the fixation property of the toner layers to a transfer material. When the difference in 1/2 method melting temperature is not greater than 10° C., preferably not less than 7° C., the adhesion between the toner layers increases (i.e., the toner layers are prevented from being separated from each other). As a result, fixability and color reproducibility of the resultant toner may not deteriorate.

The 1/2-method melting temperature of the present invention is defined as the melting temperature measured by a 1/2 flow test method of a SHIMADZU FLOWTESTER CFT-500C (manufactured by Shimadzu Corporation).

FIG. 1 is an example of a flow curve obtained by the flowtester CFT-500C. The X-axis represents a temperature and the Y-axis represents a piston stroke. As illustrated in FIG. 1, a value of a point A on the Y-axis is the midpoint between Smax and 5 min. A value of the point A on the X-axis is defined as the 1/2 method melting temperature in the present invention.

The measurement conditions are as follows:

Cylinder pressure: 10.0 kgf/cm<sup>2</sup>

Die length: 0.995 to 1.005 mm

Die orifice diameter: 0.049 to 0.051 mm

Start temperature: 50° C.

Temperature rising rate: 3.0° C./min

In order to prepare a measurement sample, 0.95 to 1.05 g of a toner is pelletized using a compacting machine including a piston having a diameter of 11.282 to 11.284 mm. The measurement sample is set in the flowtester and the 1/2 method melting temperature is measured under the above-mentioned conditions.

## 12

In the present invention, the circularity and the envelope degree of a toner are measured using a flow-type particle image analyzer FPIA-3000 (manufactured by Sysmex Corporation).

5 A typical measurement method is as follows:

(1) 0.1 to 0.5 ml of a surfactant (preferably alkylbenzene sulfonate) is included as a dispersant in 100 to 150 ml of water from which solid impurities have been removed;

(2) 0.1 to 0.5 g of a toner is added thereto and dispersed 10 using an ultrasonic dispersing machine for about 1 to 3 minutes to prepare a toner suspension liquid including 3,000 to 10,000 per 1 micro-liter of the toner particles; and

(3) the average circularity and circularity distribution of the toner are determined by the measuring instrument mentioned 15 above.

The circularity of a particle is determined by the following equation:

$$\text{Circularity} = \frac{C_s}{C_p}$$

20 wherein Cp represents the length of the circumference of the image of a particle and Cs represents the length of the circumference of a circle having the same area as that of the image of the particle.

The ratio R<sub>A</sub> (% by number) of the number of toner particles A to the total number of toner particles included in a toner and the ratio R<sub>B</sub> (% by number) of the number of toner particles B to the total number of toner particles included in the toner are determined by the following equations:

$$R_A = \frac{N_A}{N_T} \times 100$$

$$R_B = \frac{N_B}{N_T} \times 100$$

wherein N<sub>A</sub> represents the number of toner particles A included in a toner, N<sub>B</sub> represents the number of toner particles B included in the toner, and N<sub>T</sub> represents the total number of toner particles included in the toner.

The standard deviation (SD) of circularity of the toner particles A is measured with specifying the measurement ranges of particle diameter (i.e., the diameter of a circle having the same area as that of a projected image of a particle) from 0.5 μm to 200.0 μm, and of circularity greater than 0.93 and not greater than 1.00.

The average envelope degree (ED) (based on area) of the toner particles B is determined by the following equation:

$$ED \text{ (based on area)} = \frac{S_B}{H_B}$$

wherein S<sub>B</sub> and H<sub>B</sub> represent the average area and the average envelope area, respectively, of projected images of particles having a circularity of from 0.85 to 0.93.

50 As illustrated in FIG. 2, the envelope degree (based on area) is the ratio of the area (S) of a projected image of a particle to the envelope area (H) (i.e., an area of a polygon obtained by connecting convex portions of a projected image of a particle) thereof. Therefore, the ED represents a concavo-convex degree of a particle.

An example of a method for manufacturing the toner of the present invention will be explained.

At first, a binder resin (e.g., a polyol resin), a colorant (e.g., a pigment, a dye), a charge controlling agent, a wax, etc. are 60 mixed using a mixer (e.g., HENSCHEL MIXER). When a toner for use in a full-color image is prepared, a colorant master batch in which a colorant and a part of a binder resin are previously melt-kneaded is typically used, to improve dispersibility of the colorant.

65 Next, the above-prepared mixture is melt-kneaded using a kneader such as a batch-type two-roll mill, a BANBURY MIXER, a continuous double-axis extruder (e.g., TWIN

SCREW EXTRUDER KTK from Kobe Steel, Ltd., TWIN SCREW COMPOUNDER TEM from Toshiba Machine Co., Ltd., MIRACLE K.C.K from Asada Iron Works Co., Ltd., TWIN SCREW EXTRUDER PCM from Ikegai Co., Ltd., KEX EXTRUDER from Kurimoto, Ltd.), or a continuous single-axis extruder (e.g., KOKNEADER from Buss Corporation).

The kneaded mixture is then cooled and coarsely pulverized using a hammer mill, etc.

The coarsely pulverized particles are then finely pulverized using a pulverizer using an air jet and/or a mechanical pulverizer. The pulverizer using an air jet is preferably used to prepare particles having a small particle diameter. The finely pulverized particles are then classified using a classifier using a rotational flow and/or a classifier using the Coanda effect. Thus, colored particles having a desired particle diameter are produced.

In the present invention, the above-prepared colored particles are preferably subjected to a surface treatment by flowing into a thermal current. The thermal current preferably has a temperature of 50 to 100°C., more preferably 60 to 90°C., higher than the  $\frac{1}{2}$  method melting temperature of the resin used. However, the temperature of the thermal current may be controlled according to the thermal properties of the resin used. When the temperature is too much lower than the  $\frac{1}{2}$  method melting temperature of the resin, concavities and convexities on the surfaces may be smoothed. As a result, the toner particles B of the present invention may not have a desired envelope degree, and therefore ultrafine particles tend to be produced when an external impact is applied. When the temperature is too much higher than the  $\frac{1}{2}$  method melting temperature of the resin, the particles may have a true spherical shape and a narrow shape distribution. In other words, the resultant toner may not have a desired circularity distribution, resulting in deterioration of chargeability (in particular, an ability to be quickly charged) and cleanability.

The above surface treatment may be performed using an apparatus such as METEORAINBOW from Nippon Pneumatic Mfg. Co., Ltd.

The colored particles are preferably mixed with an external additive using a mixer before being subjected to the surface treatment using a thermal current, in order to prevent the colored particles from melting and forming secondary aggregations.

Specific examples of the mixers include a V-form mixer, a locking mixer, a LOEDIGE Mixer, a NAUTA MIXER, a HENSCHEL MIXER, a SUPER MIXER and the like mixers. These mixers are preferably equipped with a jacket so that the inner temperature can be controlled.

By mixing an external additive with the colored particles before being subjected to the surface treatment using a thermal current, the shapes of the colored particles can be controlled because the external additive may prevent the colored particles from melting. When the amount of the external additive is too small, the colored particles tend to have a spherical shape and a narrow particle shape distribution. Therefore, 100 parts by weight of the colored particles are preferably mixed with 0.05 to 1.0 parts by weight, more preferably 0.1 to 0.5 parts by weight, of the external additive.

If the external additive strongly fixes onto the surfaces of the colored particles and cannot exert its effect due to the thermal treatment, the external additive may be mixed with the colored particles after the thermal treatment.

The toner of the present invention can be used for a two-component developer including a toner and a magnetic car-

rier. The two-component developer preferably includes 1 to 10 parts by weight of the toner based on 100 parts by weight of the carrier.

Specific examples of the magnetic carrier include, but are not limited to, iron powders, ferrite powders, magnetite powders, and a magnetic resin carrier, which have a particle diameter of from 20 to 200  $\mu\text{m}$ . These can be covered with a covering material. Specific examples of the covering material include, but are not limited to, amino resins (e.g., urea-formaldehyde resin, melamine resin, benzoguanamine resin, urea resin, polyamide resin, epoxy resin), polyvinyl and polyvinylidene resins (e.g., acrylic resin, polymethyl methacrylate resin, polyacrylonitrile resin, polyvinyl acetate resin, polyvinyl alcohol resin, polyvinyl butyral resin), polystyrene resins (e.g., polystyrene resin, styrene-acrylic copolymer resin), halogenated olefin resins (e.g., polyvinyl chloride), polyester resins (e.g., polyethylene terephthalate resin, polybutylene terephthalate resin), polycarbonate resins, polyethylene resins, polyvinyl fluoride resins, polyvinylidene fluoride resins, polytrifluoroethylene resins, polyhexafluoropropylene resins, copolymers of vinylidene fluoride and an acrylic monomer, copolymers of vinylidene fluoride and vinyl fluoride, fluoropolymers (e.g., terpolymers of tetrafluoroethylene, vinylidene fluoride, and a non-fluoro monomer), and silicone resins.

The covering material optionally includes powders of a conductive material, if desired. Specific examples of the conductive material include, but are not limited to, carbon black, titanium oxide, tin oxide, and zinc oxide. The powders of the conductive material preferably have an average particle diameter of not greater than 1  $\mu\text{m}$ . When the particle diameter is too large, it is difficult to control the electric resistivity of the resultant carrier.

#### (Image Forming Method)

The image forming method of the present invention includes:

forming an electrostatic latent image on an electrostatic latent image bearing member;

developing the electrostatic latent image with the toner of the present invention;

transferring the toner image onto a recording medium; and

fixing the toner image on the recording medium by a non-contact fixing means.

According to the present invention, an image forming method capable of simultaneous duplex printing (copying) with a simple apparatus may be provided when a continuous transfer material is used as the recording medium in the above image forming method. In particular, the continuous transfer material drives the image bearing member by tightly winding thereon while forming an image on the transfer material, and the image is fixed by a non-contact heating method. In the present invention, "transfer material" includes a medium on which a toner image is directly transferred from an electrostatic latent image member and fixed. Specifically, papers and OHP sheets are used as the transfer material.

FIG. 3 is a schematic view illustrating an embodiment of an image forming apparatus using the image forming method of the present invention. As illustrated in FIG. 3, rotatable electrostatic latent image bearing members are preferably in a zigzag arrangement.

A supply station 30 contains a supply roller 14 on which a continuous paper 1 is wound. The continuous paper 1 is transported to a printing housing 31 containing image forming stations A, B, C, D, A', B', C', and D', each having the same configuration. The image forming stations A, B, C, and D are configured to print yellow, magenta, cyan, and black images, respectively. The image forming stations A', B', C', and D' are

15

configured to print yellow, magenta, cyan, and black images, respectively. A group of image forming stations A, B, C, and D and another group of image forming stations A', B', C', and D' each are vertically structured, resulting in reducing the footprint.

The continuous paper 1 is released from the supply roller 14 and transported upward, and subsequently passes the image forming stations. A brake 15 acts on the supply roller 14. After the continuous paper 1 passes the last image forming station D', the continuous paper 1 passes a reverse roller 17 and is transported downward, and subsequently passes an image fixing station 18, a cooling station 19, and a cutting station 20. The continuous paper 1 is cut into sheets, and the sheets are stacked on a stacker 21. The continuous paper 1 is transported by driving rollers 16a and 16b throughout the apparatus. The driving roller 16a is provided between the supply station 30 and the first image forming station A, and the driving roller 16b is provided between the cooling station 19 and the cutting station 20. The driving rollers 16a and 16b are driven by controllable motors (not shown).

FIG. 4 is a magnified schematic view illustrating an embodiment of the image forming station of the image forming apparatus illustrated in FIG. 3.

The image forming station includes a cylindrical drum 2 having a photosensitive outer surface 3. Around the cylindrical drum 2, a corotron or scorotron charger 10 configured to uniformly charge the photosensitive outer surface 3 and an irradiator 8 configured to irradiate the photosensitive outer surface 3 with a scanning laser beam or an LED array are provided along the photosensitive outer surface 3. The photosensitive outer surface 3 is irradiated in an image direction or a line direction so that the charges on the photosensitive outer surface 3 are selectively removed to form a latent image. The latent image becomes visible by contacting a developing member to the photosensitive outer surface 3 in a developing station 5. The developing station 5 includes a developing drum 4 installed controllably. The developing drum 4 may radially move toward or away from the cylindrical drum 2. Since the developing drum 4 contains a magnet in a rotating sleeve thereof, a mixture of toner particles and magnetizable carrier particles are rotated together with the rotating sleeve and form a magnetic brush on the developing drum 4. The magnetic brush contacts the photosensitive outer surface 3 on the cylindrical drum 2. The negatively charged toner particles are attracted to the irradiated portion of the photosensitive outer surface 3 due to an electric field formed between the irradiated portion and the developing member negatively biased. Thus, the latent image becomes visible, i.e., a toner image is formed.

The toner image formed on the photosensitive outer surface 3 is transferred onto the continuous paper 1 by a transfer corona charger 12.

The transfer corona charger 12 is provided opposite to the cylindrical drum 2 across the continuous paper 1. The toner particles are detached from the photosensitive outer surface 3 and attracted to the surface of the continuous paper 1 due to a high potential of the transfer corona charger 12 having reverse polarity to the toner particles. The transfer corona charger 12 functions between the continuous paper 1 and the photosensitive outer surface 3 so that a strong adsorbability is generated therebetween. Thereby, the photosensitive outer surface

16

3 rotates in synchronization with a movement of the continuous paper 1. As a result, the toner particles are tightly adhered to the surface of the continuous paper 1. However, the continuous paper 1 should not adhere to the photosensitive outer surface 3 beyond the positions where guide rollers 13 are provided. Therefore, a discharge corona charger 11 is provided on a position beyond the transfer corona charger 12 along the photosensitive outer surface 3. The discharge corona charger 11 is driven by an alternating current so that the continuous paper 1 is discharged and detached from the photosensitive outer surface 3.

The photosensitive outer surface 3 is subsequently pre-charged by a corotron or scorotron pre-charger 9. Residual toner particles remaining on the photosensitive outer surface 3 are removed by a cleaning unit 7. The cleaning unit 7 includes a cleaning brush 6 installed controllably. The cleaning brush 6 may radially move toward or away from the photosensitive outer surface 3. The cleaning brush 6 may be grounded, or detached from the photosensitive outer surface 3 and applying a potential thereto, so that the residual toner particles are attracted to the cleaning brush 6. The photosensitive outer surface 3 is prepared for a next image forming operation after being cleaned.

(Process Cartridge)

The process cartridge of the present invention includes an electrostatic latent image bearing member and a development means for developing an electrostatic latent image formed on the electrostatic latent image bearing member to form a visible image, and optionally includes a charging means, an irradiating means, a transfer means, a cleaning means, a discharge means, etc., if desired.

The process cartridge of the present invention may be detachably attached to an image forming apparatus.

FIG. 5 is a schematic view illustrating an embodiment of the process cartridge of the present invention. A process cartridge 120 includes a photoreceptor 121, a charger 122, a developing device 123, and a cleaning device 124.

Next, an image forming method of an image forming apparatus including the process cartridge 120 will be explained. The photoreceptor 121 rotates at a predetermined speed, and the surface thereof is charged by the charger 122 to reach a positive or negative predetermined potential while rotating. The photoreceptor 121 is irradiated with a light containing image information emitted by a light irradiator such as a slit irradiator and a laser beam scanning irradiator, to form an electrostatic latent image thereon. The electrostatic latent image is developed with a toner in the developing device 123, and then the toner image is transferred onto a transfer material which is timely fed from a feeding part to an area formed between the photoreceptor 121 and the transfer device so as to meet the toner images on the photoreceptor 121. The transfer material having the toner images thereon is separated from the photoreceptor 121 and transported to a fixing device so that the toner image is fixed and discharged from the image forming apparatus as a copying or a printing. After the toner image is transferred, residual toner particles remaining on the photoreceptor are removed using the cleaning device 124, and then the photoreceptor is discharged. The photoreceptor 121 is used repeatedly.

Having generally described this invention, further understanding can be obtained by reference to certain specific

## 17

examples which are provided herein for the purpose of illustration only and are not intended to be limiting. In the descriptions in the following examples, the numbers represent weight ratios in parts, unless otherwise specified.

## EXAMPLES

## Example 1

## Toner Manufacturing Example 1

The following components were mixed using a flasher.

Water 600 parts  
Wet cake of Pigment Blue 15:3 1200 parts  
(solid content: 50%)

The mixture was mixed with 1200 parts of a polyol resin (formed from a condensation reaction among an epoxy resin, bisphenol A, p-cumylphenol, and an alkylene oxide-modified epoxy resin, having a number average molecular weight (Mn) of 3000, a weight average molecular weight (Mw) of 15000, and a glass transition temperature (Tg) of 60° C.), and then kneaded for 30 minutes at 150° C. The water was removed therefrom. The kneaded mixture was drawn and cooled, and then pulverized using a pulverizer. The pulverized particles were passed through a triple-roll mill twice. Thus, a pigment master batch was prepared.

Next, the following components were mixed using a mixer.

|                                                                                                                               |            |
|-------------------------------------------------------------------------------------------------------------------------------|------------|
| Polyol resin<br>(Mn: 3,000, Mw: 15,000, Tg: 60° C.)                                                                           | 96.0 parts |
| Pigment Master Batch (prepared above)                                                                                         | 8.0 parts  |
| Charge controlling agent<br>(E-84 (a zinc salt of 3,5-di-tert-butyl salicylic acid) from<br>Orient Chemical Industries, Ltd.) | 2.0 parts  |

The mixture was melt-kneaded using a two-roll mill. The kneaded mixture was drawn and cooled, and then pulverized using a TURBO COUNTER JET MILL (from Turbo Kogyo Co., Ltd.). The pulverized particles were classified using a DS classifier (from Nippon Pneumatic Mfg. Co., Ltd.). Thus, colored particles having a volume average particle diameter of 8.8  $\mu$ m were prepared.

The following materials were mixed with 100 parts by weight of the above-prepared colored particles using a HENSCHEL MIXER.

|                                                                              |            |
|------------------------------------------------------------------------------|------------|
| Hydrophobized silica particles<br>(average primary particle diameter: 20 nm) | 0.20 parts |
| Titanium oxide particles<br>(average primary particle diameter: 15 nm)       | 0.20 parts |

A mixing operation, in which the revolution was 1890 rpm, the mixing time was 30 seconds, and the rest time was 60 seconds, was performed 5 times.

The mixed particles were thermally treated using a METEORAINBOW MR10 (from Nippon Pneumatic Mfg. Co., Ltd.) at a feed quantity of 5 kg/hr and a treatment temperature of 170° C. Thus, surface-treated colored particles were prepared.

Next, 100 parts of the surface-treated colored particles were mixed with 0.20 parts of hydrophobized silica particles (having an average primary diameter of 20 nm) using a HENSCHEL MIXER. A mixing operation, in which the revolution was 1890 rpm, the mixing time was 30 seconds, and the rest time was 60 seconds, was performed 5 times. Thus, a cyan toner (1) was prepared.

## 18

The cyan toner (1) has a volume average particle diameter of 8.8  $\mu$ m and a 1/2 method melting temperature of 110° C. The toner shape measured by FPIA-3000 is shown in Table 1. The SEM image ( $\times 1,000$ ) of the toner is shown in FIG. 6. It is clear from FIG. 6 that the cyan toner (1) includes various shaped particles (e.g., a spherical shape, a bell-like cone shape, a flat shape). Among these particles, particles being relatively not spherical (i.e., toner particles B) have a few concavities and convexities on the surfaces thereof.

10  
5  
15  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
80

19

image proportion of 1% was successively produced. The background portion of the thin line image was visually observed using a loupe and evaluated as follows.

Rank 5: No background fouling was observed.

Rank 4: Background fouling was slightly observed.

Rank 3: Background fouling was observed, but the image is acceptable.

Rank 2: Background fouling was observed, and the image is not acceptable.

Rank 1: Severe background fouling was observed.

(3) Evaluation of Durability

The charge quantity (Q/M (-μC/g)) of the developer and the image quality (e.g., transfer defect, dot reproducibility) were determined after the running test was performed, and compared with those in the initial conditions to evaluate the durability. The charge quantity of the developer was measured by a blow-off method at conditions of 23°C and 50% RR. The durability was evaluated as follows.

Rank 5: Q/M was not changed.

Rank 4: Q/M was decreased, but the image quality was not changed.

Rank 3: Q/M was decreased and background fouling was observed, but the image was acceptable.

Rank 2: Q/M was decreased and background fouling was observed, and the image was not acceptable.

Rank 1: Q/M was extremely decreased, and the image was not acceptable.

(4) Evaluation of Thermostable Preservability

A 50 ml glass container was filled with the toner, and kept in a thermostatic chamber for 20 hours at 50°C. The toner was then cooled to room temperature, and subjected to a penetrating test (based on JIS K2235-1991). The thermostable preservability was evaluated as follows.

Rank 5: The penetration depth was not less than 25 mm.

Rank 4: The penetration depth was from 20 to 25 mm.

Rank 3: The penetration depth was from 15 to 20 mm. Acceptable.

Rank 2: The penetration depth was from 10 to 15 mm. Not acceptable.

Rank 1: The penetration depth was not greater than 10 mm. Not acceptable.

Example 2

Toner Manufacturing Example 2

The following materials were mixed with 100 parts by weight of the colored particles having a volume average particle diameter of 8.8 μm, prepared in Toner Manufacturing Example 1, using a HENSCHEL MIXER.

|                                                                              |            |
|------------------------------------------------------------------------------|------------|
| Hydrophobized silica particles<br>(average primary particle diameter: 20 nm) | 0.40 parts |
| Titanium oxide particles<br>(average primary particle diameter: 15 nm)       | 0.20 parts |

A mixing operation, in which the revolution was 1890 rpm, the mixing time was 30 seconds, and the rest time was 60 seconds, was performed 5 times.

The mixed particles were thermally treated using a METEORAINBOW MR10 (from Nippon Pneumatic Mfg. Co., Ltd.) at a feed quantity of 5 kg/hr and a treatment temperature of 170°C. Thus, surface-treated colored particles were prepared.

Next, 100 parts of the surface-treated colored particles were mixed with 0.20 parts of hydrophobized silica particles

20

(having an average primary diameter of 20 nm) using a HENSCHEL MIXER. A mixing operation, in which the revolution was 1890 rpm, the mixing time was 30 seconds, and the rest time was 60 seconds, was performed 5 times. Thus, a cyan toner (2) was prepared.

The cyan toner (2) has a volume average particle diameter of 8.8 μm and a 1/2 method melting temperature of 110°C. The toner shape measured by FPIA-3000 is shown in Table 1. (Evaluation)

At first, 2325 g of the carrier (A) and 175 g of the cyan toner (2) were mixed using a TURBLER® MIXER to prepare a two-component developer having a toner concentration of 7% by weight. The two-component developer was set in a printing station of XEIKON 6000 (from Punch Graphix). The cyan toner (2) was set in a toner supplying part. A continuous paper having a basis weight of 190 g/m<sup>2</sup> was set in a paper feeding part. Images were produced at a feeding speed of 120 mm/sec and a temperature of a fixing station of 130°C.

The evaluations performed in Example 1 were repeated. The evaluation results are shown in Table 2.

Example 3

Toner Manufacturing Example 3

The following materials were mixed with 100 parts by weight of the colored particles having a volume average particle diameter of 8.8 μm, prepared in Toner Manufacturing Example 1, using a HENSCHEL MIXER.

|                                                                              |            |
|------------------------------------------------------------------------------|------------|
| Hydrophobized silica particles<br>(average primary particle diameter: 20 nm) | 0.40 parts |
| Titanium oxide particles<br>(average primary particle diameter: 15 nm)       | 0.30 parts |

A mixing operation, in which the revolution was 1890 rpm, the mixing time was 30 seconds, and the rest time was 60 seconds, was performed 5 times.

The mixed particles were thermally treated using a METEORAINBOW MR10 (from Nippon Pneumatic Mfg. Co., Ltd.) at a feed quantity of 5 kg/hr and a treatment temperature of 190°C. Thus, surface-treated colored particles were prepared.

Next, 100 parts of the surface-treated colored particles were mixed with 0.20 parts of hydrophobized silica particles (having an average primary diameter of 20 nm) using a HENSCHEL MIXER. A mixing operation, in which the revolution was 1890 rpm, the mixing time was 30 seconds, and the rest time was 60 seconds, was performed 5 times. Thus, a cyan toner (3) was prepared.

The cyan toner (3) has a volume average particle diameter of 8.8 μm and a 1/2 method melting temperature of 110°C. The toner shape measured by FPIA-3000 is shown in Table 1. (Evaluation)

At first, 2325 g of the carrier (A) and 175 g of the cyan toner (3) were mixed using a TURBLER® MIXER to prepare a two-component developer having a toner concentration of 7% by weight. The two-component developer was set in a printing station of XEIKON 6000 (from Punch Graphix). The cyan toner (3) was set in a toner supplying part. A continuous paper having a basis weight of 190 g/m<sup>2</sup> was set in a paper feeding part. Images were produced at a feeding speed of 120 mm/sec and a temperature of a fixing station of 130°C.

The evaluations performed in Example 1 were repeated. The evaluation results are shown in Table 2.

## 21

## Example 4

## Toner Manufacturing Example 4

The following materials were mixed with 100 parts by weight of the colored particles having a volume average particle diameter of 8.8  $\mu\text{m}$ , prepared in Toner Manufacturing Example 1, using a HENSCHEL MIXER.

|                                                                              |            |
|------------------------------------------------------------------------------|------------|
| Hydrophobized silica particles<br>(average primary particle diameter: 20 nm) | 0.20 parts |
| Titanium oxide particles<br>(average primary particle diameter: 15 nm)       | 0.30 parts |

A mixing operation, in which the revolution was 1890 rpm, the mixing time was 30 seconds, and the rest time was 60 seconds, was performed 5 times.

The mixed particles were thermally treated using a METEORAINBOW MR10 (from Nippon Pneumatic Mfg. Co., Ltd.) at a feed quantity of 5 kg/hr and a treatment temperature of 180° C. Thus, surface-treated colored particles were prepared.

Next, 100 parts of the surface-treated colored particles were mixed with 0.20 parts of hydrophobized silica particles (having an average primary diameter of 20 nm) using a HENSCHEL MIXER. A mixing operation, in which the revolution was 1890 rpm, the mixing time was 30 seconds, and the rest time was 60 seconds, was performed 5 times. Thus, a cyan toner (4) was prepared.

The cyan toner (4) has a volume average particle diameter of 8.8  $\mu\text{m}$  and a  $\frac{1}{2}$  method melting temperature of 110° C. The toner shape measured by FPIA-3000 is shown in Table 1. (Evaluation)

At first, 2325 g of the carrier (A) and 175 g of the cyan toner (4) were mixed using a TURBLER® MIXER to prepare a two-component developer having a toner concentration of 7% by weight. The two-component developer was set in a printing station of XEIKON 6000 (from Punch Graphix). The cyan toner (4) was set in a toner supplying part. A continuous paper having a basis weight of 190 g/m<sup>2</sup> was set in a paper feeding part. Images were produced at a feeding speed of 120 mm/sec and a temperature of a fixing station of 130° C.

The evaluations performed in Example 1 were repeated. The evaluation results are shown in Table 2.

## Example 5

## Manufacturing Example of Large-Sized Silica

A distilled methyltrimethoxysilane was heated and nitrogen gas was bubbled therein. The methyltrimethoxysilane was introduced to an oxyhydrogen flame burner together with the nitrogen gas, and burned and decomposed therein. The added amounts of the methyltrimethoxysilane, oxygen gas, hydrogen gas, and nitrogen gas were 1270 g/hr, 2.9 Nm<sup>3</sup>/hr, 2.1 Nm<sup>3</sup>/hr, and 0.58 Nm<sup>3</sup>/hr, respectively. The resultant spherical silica particles were collected using a bag filter.

Next, 1 kg of the spherical silica particles were fed into a 5-liter planetary mixer, and 10 g of pure water was added thereto while being agitated. The mixer was hermetically sealed and the mixture was agitated for 14 hours at 55° C. The mixture was cooled to room temperature, and 20 g of hexamethyldisilazane was added thereto while being agitated. The mixer was hermetically sealed again and the mixture was agitated for 24 hours. The mixture was heated to 115° C. and

## 22

aerated to nitrogen gas so that the residual raw materials and the produced ammonia were removed. Thus, large-sized silica particles were prepared.

The large-sized silica particles have a number average primary particle diameter (R) of 110 nm, a standard deviation ( $\sigma$ ) of primary particle diameter of 50 nm, a SF-1 of 120, and a SF-2 of 109.

## Toner Manufacturing Example 5

The following materials were mixed with 100 parts by weight of the surface-treated colored particles prepared in Toner Manufacturing Example 4 using a HENSCHEL MIXER.

|                                                                              |            |
|------------------------------------------------------------------------------|------------|
| Hydrophobized silica particles<br>(average primary particle diameter: 20 nm) | 0.10 parts |
| Large-sized silica particles<br>(average primary particle diameter: 110 nm)  | 0.20 parts |

A mixing operation, in which the revolution was 1890 rpm, the mixing time was 30 seconds, and the rest time was 60 seconds, was performed 5 times. Thus, a cyan toner (5) was prepared.

The cyan toner (5) has a volume average particle diameter of 8.8  $\mu\text{m}$  and a  $\frac{1}{2}$  method melting temperature of 110° C. The toner shape measured by FPIA-3000 is shown in Table 1. (Evaluation)

At first, 2325 g of the carrier (A) and 175 g of the cyan toner (5) were mixed using a TURBLER® MIXER to prepare a two-component developer having a toner concentration of 7% by weight. The two-component developer was set in a printing station of XEIKON 6000 (from Punch Graphix). The cyan toner (5) was set in a toner supplying part. A continuous paper having a basis weight of 190 g/m<sup>2</sup> was set in a paper feeding part. Images were produced at a feeding speed of 120 mm/sec and a temperature of a fixing station of 130° C.

The evaluations performed in Example 1 were repeated. The evaluation results are shown in Table 2.

## Comparative Example 1

## Toner Manufacturing Example 6

The following components were mixed using a flasher.

|                                                       |            |
|-------------------------------------------------------|------------|
| Water                                                 | 600 parts  |
| Wet cake of Pigment Blue 15:3<br>(solid content: 50%) | 1200 parts |

The mixture was mixed with 1200 parts of a polyol resin (having a number average molecular weight (Mn) of 3000, a weight average molecular weight (Mw) of 15000, and a glass transition temperature (Tg) of 60° C.), and then kneaded for 30 minutes at 150° C. The water was removed therefrom. The kneaded mixture was drawn and cooled, and then pulverized using a pulverizer. The pulverized particles were passed through a triple-roll mill twice. Thus, a pigment master batch was prepared.

Next, the following components were mixed using a mixer.

|                                                     |            |
|-----------------------------------------------------|------------|
| Polyol resin<br>(Mn: 3,000, Mw: 15,000, Tg: 60° C.) | 96.0 parts |
| Pigment Master Batch (prepared above)               | 8.0 parts  |

|                                                                                                                               |           |
|-------------------------------------------------------------------------------------------------------------------------------|-----------|
| Charge controlling agent<br>(E-84 (a zinc salt of 3,5-di-tert-butyl salicylic acid) from<br>Orient Chemical Industries, Ltd.) | 2.0 parts |
|-------------------------------------------------------------------------------------------------------------------------------|-----------|

The mixture was melt-kneaded using a two-roll mill. The kneaded mixture was drawn and cooled, and then pulverized using a TURBO COUNTER JET MILL (from Turbo Kogyo Co., Ltd.). The pulverized particles were classified using a DS classifier (from Nippon Pneumatic Mfg. Co., Ltd.). Thus, colored particles having a volume average particle diameter of 8.8  $\mu\text{m}$  were prepared.

The following materials were mixed with 100 parts by weight of the above-prepared colored particles using a HENSCHEL MIXER.

|                                                                              |            |
|------------------------------------------------------------------------------|------------|
| Hydrophobized silica particles<br>(average primary particle diameter: 20 nm) | 0.40 parts |
| Titanium oxide particles<br>(average primary particle diameter: 15 nm)       | 0.20 parts |

A mixing operation, in which the revolution was 1890 rpm, the mixing time was 30 seconds, and the rest time was 60 seconds, was performed 5 times. Thus, a cyan toner (6) was prepared.

The cyan toner (6) has a volume average particle diameter of 8.8  $\mu\text{m}$  and a  $\frac{1}{2}$  method melting temperature of 109°C. The toner shape measured by FPIA-3000 is shown in Table 1. (Evaluation)

At first, 2325 g of the carrier (A) and 175 g of the cyan toner (6) were mixed using a TURBLER® MIXER to prepare a two-component developer having a toner concentration of 7% by weight. The two-component developer was set in a printing station of XEIKON 6000 (from Punch Graphix). The cyan toner (6) was set in a toner supplying part. A continuous paper having a basis weight of 190 g/m<sup>2</sup> was set in a paper feeding part. Images were produced at a feeding speed of 120 mm/sec and a temperature of a fixing station of 130°C.

The evaluations performed in Example 1 were repeated. The evaluation results are shown in Table 2.

#### Comparative Example 2

#### Toner Manufacturing Example 7

In a reaction vessel, 750 parts of ion-exchanged water and 500 parts of a 0.1 M aqueous solution of Na<sub>3</sub>PO<sub>4</sub> were contained. The mixture was heated to 65°C. and agitated using TK HOMO MIXER® (from Tokushu Kika Kogyo Co., Ltd.) at a revolution of 12000 rpm. Next, 85 parts of a 1.5 M aqueous solution of CaCl<sub>2</sub> was gradually added thereto. Thus, an aqueous medium containing Ca<sub>3</sub>(PO<sub>4</sub>)<sub>2</sub> was prepared.

In another reaction vessel, the following components were contained.

|                                                                          |             |
|--------------------------------------------------------------------------|-------------|
| Styrene                                                                  | 165.0 parts |
| n-Butyl acrylate                                                         | 34.0 parts  |
| Colorant (C.I. Pigment Blue 15:3)                                        | 13.0 parts  |
| Polar resin (Polyester resin)                                            | 15.0 parts  |
| Charge controlling agent<br>(E-84 from Orient Chemical Industries, Ltd.) | 3.0 parts   |
| Cross-linker (Divinylbenzene)                                            | 0.4 parts   |

The mixture was heated to 65°C. and mixed using TK HOMO MIXER® (from Tokushu Kika Kogyo Co., Ltd.) at a revolution of 12000 rpm.

Further, 12 parts of a polymerization initiator 2,2'-azobis (2,4-dimethylvaleronitrile) was dissolved therein. Thus, a monomer composition was prepared.

The monomer composition was poured into the aqueous medium prepared above, and then the mixture was agitated for 5 minutes at 65°C. using TK HOMO MIXER® (from Tokushu Kika Kogyo Co., Ltd.) at a revolution of 10000 rpm under N<sub>2</sub> atmosphere so that the monomer composition was granulated. The mixture was further subjected to a reaction for 6 hours at 65°C. and 10 hours at 85°C. while agitated by paddle agitation blades.

After the reaction was terminated, the reaction vessel was cooled. Hydrochloric acid was added thereto, and calcium phosphate was dissolved therein. The mixture was filtered, washed with water, and dried. Thus, colored particles were prepared.

The following materials were mixed with 100 parts by weight of the above-prepared colored particles using a HENSCHEL MIXER.

|                                                                              |            |
|------------------------------------------------------------------------------|------------|
| Hydrophobized silica particles<br>(average primary particle diameter: 20 nm) | 0.40 parts |
| Titanium oxide particles<br>(average primary particle diameter: 15 nm)       | 0.20 parts |

A mixing operation, in which the revolution was 1890 rpm, the mixing time was 30 seconds, and the rest time was 60 seconds, was performed 5 times. Thus, a cyan toner (7) was prepared.

The cyan toner (7) has a volume average particle diameter of 7.5  $\mu\text{m}$  and a  $\frac{1}{2}$  method melting temperature of 115°C. The toner shape measured by FPIA-3000 is shown in Table 1. (Evaluation)

At first, 2325 g of the carrier (A) and 175 g of the cyan toner (7) were mixed using a TURBLER® MIXER to prepare a two-component developer having a toner concentration of 7% by weight. The two-component developer was set in a printing station of XEIKON 6000 (from Punch Graphix). The cyan toner (7) was set in a toner supplying part. A continuous paper having a basis weight of 190 g/m<sup>2</sup> was set in a paper feeding part. Images were produced at a feeding speed of 120 mm/sec and a temperature of a fixing station of 130°C.

The evaluations performed in Example 1 were repeated. The evaluation results are shown in Table 2.

#### Comparative Example 3

The following materials were mixed using a HENSCHEL MIXER.

|                                                                              |            |
|------------------------------------------------------------------------------|------------|
| Colored particles prepared in Toner Manufacturing Example                    | 30.0 parts |
| Colored particles prepared in Toner Manufacturing Example                    | 70.0 parts |
| Hydrophobized silica particles<br>(average primary particle diameter: 20 nm) | 0.40 parts |
| Titanium oxide particles<br>(average primary particle diameter: 15 nm)       | 0.20 parts |

A mixing operation, in which the revolution was 1890 rpm, the mixing time was 30 seconds, and the rest time was 60 seconds, was performed 5 times. Thus, a cyan toner (8) was prepared.

The cyan toner (8) has a volume average particle diameter of 7.9  $\mu\text{m}$  and a  $\frac{1}{2}$  method melting temperature of 113°C. The toner shape measured by FPIA-3000 is shown in Table 1.

## (Evaluation)

At first, 2325 g of the carrier (A) and 175 g of the cyan toner (8) were mixed using a TURBLER® MIXER to prepare a two-component developer having a toner concentration of 7% by weight. The two-component developer was set in a printing station of XEIKON 6000 (from Punch Graphix). The cyan toner (8) was set in a toner supplying part. A continuous paper having a basis weight of 190 g/m<sup>2</sup> was set in a paper feeding part. Images were produced at a feeding speed of 120 mm/sec and a temperature of a fixing station of 130° C.

The evaluations performed in Example 1 were repeated. The evaluation results are shown in Table 2.

TABLE 1

|       | Toner particles A                                 |                    | Toner particles B                                 |                     |                                          |
|-------|---------------------------------------------------|--------------------|---------------------------------------------------|---------------------|------------------------------------------|
|       | R <sub>A</sub> <sup>(*)</sup><br>(% by<br>number) | SD <sup>(**)</sup> | R <sub>B</sub> <sup>(*)</sup><br>(% by<br>number) | ED <sup>(***)</sup> | ½ method melting<br>temperature<br>(°C.) |
| Ex. 1 | 71.0                                              | 0.014              | 29.0                                              | 0.941               | 110                                      |
| Ex. 2 | 72.5                                              | 0.025              | 27.5                                              | 0.940               | 110                                      |
| Ex. 3 | 93.5                                              | 0.025              | 6.5                                               | 0.950               | 110                                      |
| Ex. 4 | 74.8                                              | 0.014              | 25.2                                              | 0.948               | 110                                      |
| Ex. 5 | 74.8                                              | 0.014              | 25.2                                              | 0.948               | 110                                      |
| Comp. | 58.0                                              | 0.017              | 37.0                                              | 0.936               | 109                                      |
| Ex. 1 |                                                   |                    |                                                   |                     |                                          |
| Comp. | 97.7                                              | 0.012              | 2.3                                               | 0.966               | 115                                      |
| Ex. 2 |                                                   |                    |                                                   |                     |                                          |
| Comp. | 83.5                                              | 0.020              | 16.5                                              | 0.938               | 113                                      |
| Ex. 3 |                                                   |                    |                                                   |                     |                                          |

(\*)R<sub>A</sub>, R<sub>B</sub>: Ratio of the number of toner particles A and B, respectively, to the total number of toner particles included in a toner

(\*\*) SD: Standard deviation of circularity of toner particles A

(\*\*\*) ED: Average envelope degree (based on area) of toner particles B

TABLE 2

|       | Smudge<br>on edge<br>portion | Background<br>fouling | Durability | Thermostable<br>preservability |  |
|-------|------------------------------|-----------------------|------------|--------------------------------|--|
| Ex. 1 | 5                            | 5                     | 4          | 3                              |  |
| Ex. 2 | 5                            | 5                     | 4          | 3                              |  |
| Ex. 3 | 5                            | 4                     | 5          | 3                              |  |
| Ex. 4 | 5                            | 4                     | 5          | 3                              |  |
| Ex. 5 | 5                            | 4                     | 5          | 5                              |  |
| Comp. | 1                            | 2                     | 1          | 4                              |  |
| Ex. 1 |                              |                       |            |                                |  |
| Comp. | 3                            | 1                     | 5          | 2                              |  |
| Ex. 2 |                              |                       |            |                                |  |
| Comp. | 2                            | 2                     | 2          | 3                              |  |
| Ex. 3 |                              |                       |            |                                |  |

Additional modifications and variations of the present invention are possible in light of the above teachings. It is therefore to be understood that within the scope of the appended claims the invention may be practiced other than as specifically described herein.

This document claims priority and contains subject matter related to Japanese Patent Applications No. 2006-311162, 2007-236088 and 2007-243514, filed on Nov. 17, 2006, Sep. 12, 2007 and Sep. 20, 2007, respectively, the entire contents of which are herein incorporated by reference.

What is claimed is:

1. A toner, comprising:

toner particles A having a circularity of greater than 0.93 and not greater than 1.00; and

toner particles B having a circularity of from 0.85 to 0.93, wherein the following relationships are satisfied:

$$70 \leq R_A \leq 95$$

$$5 \leq R_B \leq 30$$

$$0.014 \leq SD \leq 0.025$$

$$0.940 \leq ED \leq 0.950$$

10 wherein R<sub>A</sub> (% by number) represents a ratio of a number of the toner particles A to a total number of toner particles included in the toner, R<sub>B</sub> (% by number) represents a ratio of a number of the toner particles B to the total number of toner particles included in the toner, SD represents a standard deviation of circularity of the toner particles A, and ED represents an average envelope degree of the toner particles B, wherein the toner particles A and the toner particles B are obtained by conducting a surface treatment by mixing colored particles with first silica particles and then flowing into a thermal current, and

20 wherein the amount of the first silica particles is 0.20 part by mass to 0.40 part by mass relative to 100 parts by mass of the colored particles.

25 2. The toner according to claim 1, further comprising second silica particles having a number average primary particle diameter (R) of from 80 to 200 nm.

30 3. The toner according to claim 2, wherein the second silica particles have a shape factor SF-1 of from 100 to 130 and a shape factor SF-2 of from 100 to 125, and the following relationship is satisfied:

$$R/4 \leq \sigma \leq R$$

35 wherein R represents a number average primary particle diameter of the second silica particles and  $\sigma$  represents a standard deviation of particle diameter distribution of the second silica particles.

40 4. The toner according to claim 1, wherein both the toner particles A and B comprise a polyol resin and the toner has a ½ method melting temperature of from 100 to 115° C.

45 5. The toner according to claim 2, wherein both the toner particles A and B comprise a polyol resin and the toner has a ½ method melting temperature of from 100 to 115° C.

50 6. The toner according to claim 3, wherein both the toner particles A and B comprise a polyol resin and the toner has a ½ method melting temperature of from 100 to 115° C.

55 7. An image forming method, comprising: forming an electrostatic latent image on an electrostatic latent image bearing member; developing the electrostatic latent image with the toner according to claim 1 to form a toner image; transferring the toner image onto a recording medium; and fixing the toner image on the recording medium by a non-contact fixing means.

60 8. An image forming method according to claim 7, wherein the toner further comprises second silica particles having a number average primary particle diameter (R) of from 80 to 200 nm.

65 9. An image forming method according to claim 8, wherein the silica particles have a shape factor SF-1 of from 100 to 130 and a shape factor SF-2 of from 100 to 125, and the following relationship is satisfied:

$$R/4 \leq \sigma \leq R$$

70 wherein R represents a number average primary particle diameter of the silica particles and  $\sigma$  represents a standard deviation of particle diameter distribution of the silica particles.

27

10. An image forming method according to claim 7, wherein both the toner particles A and B comprise a polyol resin and the toner has a ½ method melting temperature of from 100 to 115° C.

11. An image forming method according to claim 8, wherein both the toner particles A and B comprise a polyol resin and the toner has a ½ method melting temperature of from 100 to 115° C.

12. An image forming method according to claim 9, wherein both the toner particles A and B comprise a polyol resin and the toner has a ½ method melting temperature of from 100 to 115° C.

13. A process cartridge detachably attachable to an image forming apparatus, comprising:

an electrostatic latent image bearing member configured to bear an electrostatic latent image; and a development device which includes the toner according to claim 1 and configured to develop the electrostatic latent image with the toner.

14. A process cartridge according to claim 13, wherein the toner further comprises second silica particles having a number average primary particle diameter (R) of from 80 to 200 nm.

5

28

15. A process cartridge according to claim 14, wherein the second silica particles have a shape factor SF-1 of from 100 to 130 and a shape factor SF-2 of from 100 to 125, and the following relationship is satisfied:

$$R/4 \leq \sigma \leq R$$

wherein R represents a number average primary particle diameter of the second silica particles and  $\sigma$  represents a standard deviation of particle diameter distribution of the second silica particles.

16. A process cartridge according to claim 13, wherein both the toner particles A and B comprise a polyol resin and the toner has a ½ method melting temperature of from 100 to 115° C.

17. A process cartridge according to claim 14, wherein both the toner particles A and B comprise a polyol resin and the toner has a ½ method melting temperature of from 100 to 115° C.

18. A process cartridge according to claim 15, wherein both the toner particles A and B comprise a polyol resin and the toner has a ½ method melting temperature of from 100 to 115° C.

\* \* \* \* \*